

- [54] **ABRASION RESISTANT CELLULOSIC FABRICS CONTAINING GRAFT POLYMERIZED DIETHYLPHOSPHATOETHYLMETHACRYLATE AND/OR DIETHYLPHOSPHATO-ETHYL ACRYLATE**
- [75] Inventors: **W. James Brickman**, Philadelphia; **Robert W. Faessinger**, Media, both of Pa.
- [73] Assignee: **Scott Paper Company**, Philadelphia, Pa.
- [22] Filed: **Oct. 2, 1974**
- [21] Appl. No.: **511,176**
- [52] U.S. Cl..... 260/17.4 GC; 8/116 R; 8/116 P; 8/194; 8/DIG. 18; 117/139.5 A
- [51] Int. Cl.<sup>2</sup>..... C08L 1/02; D06M 13/32; D06M 13/44
- [58] Field of Search.. 260/17.4 GC; 8/116 R, 116 P, 8/194, DIG. 18

[56] **References Cited**

UNITED STATES PATENTS

|           |         |                        |          |
|-----------|---------|------------------------|----------|
| 2,955,015 | 10/1960 | Segro et al.....       | 8/116    |
| 3,558,596 | 1/1971  | Demott .....           | 8/116    |
| 3,821,137 | 6/1974  | Lishevskaya et al..... | 260/17.4 |

FOREIGN PATENTS OR APPLICATIONS

|         |        |              |           |
|---------|--------|--------------|-----------|
| 736,508 | 6/1966 | Canada ..... | 117/139.5 |
|---------|--------|--------------|-----------|

*Primary Examiner*—Melvin Goldstein  
*Assistant Examiner*—Edward Woodberry  
*Attorney, Agent, or Firm*—Nicholas J. DeBenedictis; John W. Kane, Jr.

[57] **ABSTRACT**

The abrasion resistance of cellulose and cellulose containing fabrics such as cotton and rayon is improved by graft copolymerizing diethylphosphatoethylmethacrylate and/or diethylphosphatoethylacrylate onto the cellulosic substrate.

**8 Claims, No Drawings**

**ABRASION RESISTANT CELLULOSIC FABRICS  
CONTAINING GRAFT POLYMERIZED  
DIETHYLPHOSPHATOETHYLMETHACRYLATE  
AND/OR DIETHYLPHOSPHATO-ETHYL  
ACRYLATE**

**BACKGROUND OF THE INVENTION**

**1. Field of the Invention**

This invention relates to improving the abrasion resistance of cellulose fabrics and cellulose-containing fabrics such as cotton, rayon and cotton-synthetic blends. This invention also relates to imparting durable flame retardant characteristics to such fabrics.

**2. Description of the Prior Art**

The graft copolymerization of cellulosic fabrics usually reduces the abrasion resistance and strength of the grafted substrate and this reduction becomes more pronounced as the quantity of polymer grafted onto the fabric is increased. The graft copolymerization of cellulosic fabrics with conventional fire retardant monomers such as vinylidene chloride, allyl phosphates, bis(chloroethyl)vinylphosphonate and the like while imparting some degree of permanent fire retardancy to the grafted substrate requires substantial additions of polymer onto the fiber (add-on) for effective fire retardancy which unfortunately adversely affects the abrasion resistance of the grafted substrate. Highly halogenated polymers are particularly detrimental to abrasion resistance due to the hydrolytic effect upon the cellulose of the relatively labile halogen atom while a multi-functional vinyl molecule tends to embrittle, thus weakening the grafted fabric.

The addition of resinous materials to fabrics to impart a permanent press character to the fabric is known to drastically reduce the abrasion resistance of a cellulosic fabric and as a result, the use of cotton-polyester blend fabrics or other cellulosic-synthetic fiber blends have become popular for such permanent press treatments in an attempt to compensate for the loss in abrasion resistance and strength incurred by the resin treatment on the cellulosic fiber.

Conventional durable press resins in current use do not impart any significant fire retardancy to the cellulosic substrate. Cellulosic textiles are very flammable especially when in a napped or brushed form. Many treatments, in addition to graft copolymerization discussed above, have been devised for adding flame retardant characteristics to cellulosic textiles with varying degrees of permanency. Chemicals rich in phosphorous and nitrogen have been devised which when padded onto the cellulosic substrate and subsequently cured with heat imparts a flame retardant property with some degree of permanence (durable). Flame retardancy achieved by this technique usually is durable to a number of home launderings but the fabric so treated suffers from a loss of hand, and a reduction in abrasion resistance and strength through a stiffening of the textile structure.

The monomers, diethylphosphatoethylmethacrylate and diethylphosphatoethylacrylate, have been disclosed in Canadian Patent No. 736,508 issued June 14, 1966 entitled "Dialkyl Phosphatoalkyl Acrylates and Methacrylates and Processes for Preparing Same". At page 18 of the British patent there is disclosed the use of such compounds for imparting exceptionally good flame-retardant properties to textile and like materials such as leather when the latter are impregnated there-

with. This Canadian patent does not suggest a graft copolymerization of the compounds onto cellulosic fabrics nor the significant improvement in abrasion resistance discovered and disclosed herein.

5

2

**SUMMARY OF THE INVENTION**

Cellulosic fabrics having improved abrasion resistance comprise the graft copolymer of a cellulosic fabric and a monomer selected from the group consisting of diethylphosphatoethylmethacrylate and/or diethylphosphatoethylacrylate. Durable press fabrics having abrasion resistance comparable to untreated cellulosic fabrics are provided by capping said graft copolymerized fabric with a permanent press resin. The graft copolymerized fabric provided also has outstanding fire retardancy.

**DESCRIPTION OF THE PREFERRED EMBODIMENTS**

20 The graft copolymerization of cellulosic materials (fibers or fabrics) with vinyl compounds is well known in the art. The graft copolymerization of cellulosic substrates with diethylphosphatoethylmethacrylate or diethylphosphatoethylacrylate can be accomplished by 25 any of the various methods appearing in the literature for graft copolymerizing. Examples of suitable graft copolymerizing processes for making the fabrics and fibers of the present invention are disclosed in U.S. Pat. No. 3,359,224, entitled "Thioated Cellulosic Amylaceous Substrates-Ethylenically Unsaturated Monomer Graft Copolymer", issued to R. W. Faessinger et al.; U.S. Pat. No. 2,955,015, entitled "Graft Copolymerization of Certain Esters of Acrylic Acids With Cellular Substrate", issued to N. Segrow et al.; and U.S. Pat. No. 3,083,118, entitled "Method Of Depositing A Polymer of Olefinically Unsaturated Monomer Within A Polymeric Material And The Resulting Product", issued to D. J. Bridgeford, which disclosures are incorporated herein by reference with respect to teaching methods 30 for graft copolymerization. Many other publications demonstrate various in situ addition of polymers by pad-on-and-cure techniques initiated by heat or high energy irradiation and are well known to those skilled in the art.

35 40 45 Typical cellulosic fabrics are cotton, rayon and linen fabrics. The term "fabric" as used herein includes substrates in a woven, nonwoven, molded or knitted form since the shape and structural characteristics of the fabric are not significant. The cellulosic fabric may be a blend of cellulosic fibers with non-cellulosic fibers such as synthetic fibers (e.g., nylon and polyester) provided the cellulosic fiber constitutes at least about 50% of the fibers by weight. The term "cellulosic fiber" is used herein for its common meaning and includes both 50 55 regenerated cellulosic fibers such as rayon and natural cellulosic fibers such as cotton fibers and fibers obtained from other plants.

By durable (permanent) press resin is meant any of the innumerable resin systems composed of nitrogen-containing compounds such as trimethylolmelamine, hexamethoxymethylmelamine, dimethyloldihydroxyethylene urea, variously substituted dimethyl triazones, bismethoxymethyl urea and the like which are readily available to textile finishers under a variety of trade names. The present invention does not include the discovery of durable (permanent) press resins but comprises in part the discovery of the compatibility of such resins with the abrasion resistant fibers and fabrics

disclosed herein. No special precautions are needed in the application of these durable press resins on the graft copolymerized fabrics of this invention and the resin manufacturer's directions for use are to be followed. The amount of resin required will be dictated by the degree of durable press required in the finished fabric and the instructions of the manufacturer. Such resins can be added onto the grafted fabric and are usually employed in percentages of from about 0.5% to about 15%.

Monomers suitable for use in the present invention are

1. diethylphosphatoethylacrylate, which has the following formula:



and,

2. diethylphosphatoethyl methacrylate, which has the following formula:



In addition to increasing the abrasion resistance of cellulosic fabrics, the monomers also impart durable flame retardancy to the fabric. The flame retardancy is more durable than the flame retardancy obtained when cellulosic fabrics are impregnated with the monomers rather than graft copolymerized with the monomers.

The amount of the monomer, diethylphosphatoethylmethacrylate, or diethylphosphatoethylacrylate, to be used will vary depending on the degree of abrasion resistance and/or the degree of fire retardancy desired. The grafted cellulosic substrate preferably contains enough polymer, poly(diethylphosphatoethylmethacrylate) and/or poly(diethylphosphatoethylacrylate) to yield a phosphorus content of from about 0.5 to 10% by weight of the graft copolymerized fabric based upon the weight of cellulosic fibers in the fabric. However, the more preferred range is from about 1.5 to 3.5% by weight phosphorus on the fabric, with the lower value preferred when durable press resins are to be used and the upper value when used alone on an all cellulosic substrate.

Diethylphosphatoethylmethacrylate is the preferred monomer because of its greater stability and higher grafting efficiency.

In order to describe the present invention so that it may be more clearly understood, the following examples are set forth. These examples are set forth primarily for the purposes of illustration, and any specific enumeration of detail contained therein should not be interpreted as a limitation of the broad concept of this invention. All proportions given herein are by weight unless indicated otherwise.

### EXAMPLE 1

Four specimens (1, 2, 3 and 4) of cotton flannelette having a basis weight of  $3\frac{1}{2}$  oz./yd.<sup>2</sup> were graft copolymerized with diethylphosphatoethylmethacrylate to various polymer add-ons onto the fabric by the method

of Faessinger et al. described in U.S. Pat. No. 3,359,224. One grafted specimen (4) and an ungrafted control (A) were given an after-treatment with American Cyanamid's Aerotex M-3 (trimethylolmelamine) to impart durable press character to the fabric. All specimens, including one untreated control (B), were subjected to a single standard home laundering and to the Tabor Abrasion Test (H-18 abrasion wheels) and the number of cycles to failure was noted. The percentage of polymer and/or resin addition to the specimens and the abrasion test results are given in Table I.

### EXAMPLE II

15 Two specimens (5 and 6) of cotton flannelette fabric having a basis weight of  $3\frac{1}{2}$  oz./yd.<sup>2</sup> were graft copolymerized with diethylphosphatoethylmethacrylate to about 12% polymer content by the method of Segrow, et al, described in U.S. Pat. No. 2,955,015. One grafted specimen (6) and an ungrafted control (C) were given  
20 an after-treatment with Aerotex M-3 (American Cyanamid, trimethylolmelamine) to impart durable press character to the fabric. The specimens and one untreated, ungrafted control specimen (D), were laundered and then subjected to the Tabor Abrasion (H-18  
25 abrasion wheels) test and the number of cycles to failure was noted. The percentage of polymer and/or resin addition and the results are given in Table I.

### EXAMPLE III

30 Two specimens (7 and 8) of cotton flannelette having a basis weight of  $3\frac{1}{2}$  oz./yd.<sup>2</sup> were graft copolymerized with diethylphosphatoethylmethacrylate to various polymer add-ons by the method of Bridgeford described in U.S. Pat. 3,083,118. One grafted specimen (8) and an ungrafted control specimen (E) were given an after-treatment with Aerotex M-3 (American Cyanamid, triethanolmelamine) to impart durable press character to the fabric. The specimens, and one untreated, ungrafted control specimen (F), were subjected to the 40 Tabor Abrasion test (H-18 abrasion wheel) after a single home-type laundering, and the number of cycles to failure was noted. The percentage of polymer and/or resin addition and the results are given in Table I.

#### EXAMPLE IV

Two specimens of rayon challis fabric (9 and 10), having a basis weight of 4 oz./yd.<sup>2</sup>, were grafted by first padding on a sufficient quantity of a bath composed of an emulsion consisting of diethylphosphatoethylmethacrylate and a catalytic amount of potassium persulfate, to yield a grafted polymer add-on of about 17.5%; then drying and curing the specimens in an oven at 250°F. for about 15 minutes. After a post-polymerization wash in sodium bisulfite solution followed with fresh water rinse, one grafted specimen (10) and an ungrafted specimen (G) were given an after-treatment with Aerotex M-3 (American Cyanamid, trimethylolmelamine) to impart durable press character to the treated fabric. The specimens, and one untreated ungrafted control specimen (H), were subjected to the Tabor Abrasion test (H-18 abrasion wheels) and the number of cycles to failure noted. The percentage of polymer and/or resin addition and the results are given in Table I.

**EXAMPLE V**

Several specimens (11 and 12) of cotton/polyester blend (65/35) fabric having a basis weight of 4 oz./yd.<sup>2</sup>

were grafted with diethylphosphatoethylmethacrylate to a polymer add-on of about 27% by the method of Faessinger, et al, described in U.S. Pat. No. 3,359,224. One grafted specimen (12) and an ungrafted control specimen (I) were given an after-treatment with Aerotex M-3 (American Cyanamid, trimethylolmelamine) to impart durable press character to the fabric. The specimens, and an untreated ungrafted control specimen (J), were subjected to the Tabor Abrasion test (H-18 abrasion wheels) and the number of cycles to failure was noted. The percentage of polymer and/or resin addition and the results are given in Table I.

#### EXAMPLE VI

Two specimens, (13 and 14) of cotton flannelette having a basis weight of 3½ oz./yd.<sup>2</sup> were graft copolymerized with diethylphosphatoethylmethacrylate as described in Example I. Specimen 14 and control speci-

men (M) were after-treated with Aerotex P-225 resin (American Cyanamid, hexamethoxymethylmelamine) in the manufacturer's prescribed manner. Portions of the specimens and one untreated, ungrafted control specimen (N) were subjected to the Tabor Abrasion test (H-18 abrasion wheel) after a single homestyle laundering and the number of cycles to failure was noted. The percentage of polymer and/or resin addition and the results are reported in Table I.

10

#### EXAMPLE VIII

Portions of the specimens of Example VII after the single homestyle laundering were tested for flame retardancy according to the U.S. Department of Commerce procedure DOC FF 3-71. Control specimens M and N burned their entire length while specimen 15 self-extinguished after 2.2 seconds with a char length of 3.6 inches.

TABLE I

| Example No. | Specimen No. | Percent Resin | Polymer Add-On | Fail Cycles |
|-------------|--------------|---------------|----------------|-------------|
| I           | 1            | —             | 19.1           | 78.2        |
| I           | 2            | —             | 24.8           | 78.4        |
| I           | 3            | —             | 33.1           | 94.8        |
| I           | 4            | 7.3           | 19.1           | 77.4        |
| I           | A            | 5.7           | —              | 42.5        |
| I           | B            | —             | Control        | 76          |
| II          | 5            | —             | 12             | 119         |
| II          | 6            | 7.1           | 12             | 86          |
| II          | C            | 7.3           | —              | 69          |
| II          | D            | —             | Control        | 96          |
| III         | 7            | —             | 21             | 191         |
| III         | 8            | 60            | 21             | 74          |
| III         | E            | 7.3           | —              | 69          |
| III         | F            | —             | Control        | 96          |
| IV          | 9            | —             | 17.5           | 69          |
| IV          | 10           | 5.8           | 17.5           | 53          |
| IV          | G            | 7.5           | —              | 43          |
| IV          | H            | —             | Control        | 66          |
| V           | 11           | —             | 27             | 73          |
| V           | 12           | 5.0           | 27             | 71          |
| V           | I            | 6.0           | —              | 53          |
| V           | J            | —             | Control        | 65          |
| VII         | 15           | 8.2           | 24.5           | 66          |
| VII         | M            | 4.0           | —              | 30          |
| VII         | N            | —             | Control        | 101         |

men (K) were after-treated with Permafresh 183 resin (Sun Chemical Company, dimethyloldihydroxyethylene urea) in the manufacturer's prescribed manner. The treated specimens and an untreated control specimen (L) were repeatedly laundered and the laundering abrasion resistance as measured by the loss in weight was observed after 1 and 50 launderings. The loss in dry fill breaking stress of each specimen was observed. The results are reported in Table II.

TABLE II

| Specimen | Launder Cycles | Laundring Abrasion Wt. Loss % | Breaking Stress % of Control |
|----------|----------------|-------------------------------|------------------------------|
| L        | 1              | 1.9%                          | 100.0                        |
| L        | 50             | 4.9%                          | 90.0                         |
| K        | 1              | 7.2%                          | 43.5                         |
| K        | 50             | 21.2%                         | 37.3                         |
| 13       | 1              | 0.1%                          | 92.6                         |
| 13       | 50             | 3.1%                          | 73.4                         |
| 14       | 1              | 1.4%                          | 58.6                         |
| 14       | 50             | 7.0%                          | 47.6                         |

#### EXAMPLE VII

A specimen (15) of cotton flannelette having a basis weight of 3½ oz./yd.<sup>2</sup> were graft copolymerized with diethylphosphatoethylmethacrylate as described in Example I. Specimen 15 and an ungrafted control speci-

men (K) were after-treated with Aerotex P-225 resin (American Cyanamid, hexamethoxymethylmelamine) in the manufacturer's prescribed manner. Portions of the specimens and one untreated, ungrafted control specimen (N) were subjected to the Tabor Abrasion test (H-18 abrasion wheel) after a single homestyle laundering and the number of cycles to failure was noted. The percentage of polymer and/or resin addition and the results are reported in Table I.

45

What is claimed is:

1. A cellulosic fabric having improved abrasion resistance comprising a cellulosic fabric graft copolymerized with a monomer selected from the group consisting of ethylphosphatoethylmethacrylate and ethylphosphatoethylacrylate.

50 2. The cellulosic fabric of claim 1 having an amount of monomer graft copolymerized onto the cellulosic fabric to result in a phosphorous content of from 0.5% to 10% based upon the weight of cellulose fibers in the fabric.

55 3. The abrasion resistant fabric of claim 1 in which the cellulosic fabric is a blend of cellulosic fibers with non-cellulosic fibers in which the cellulosic fibers comprise at least about 50% of the fibers in the fabric.

4. The abrasion resistant cellulosic fabric of claim 1 further comprising a durable press resin added onto the cellulosic fabric after graft copolymerization.

60 5. The abrasion resistant cellulosic fabric of claim 1 in which the fabric is a cotton containing fabric.

6. The abrasion resistant cellulosic fabric of claim 1 in which the fabric is a rayon containing fabric.

7. The abrasion resistant cellulosic fabric of claim 1 in which the fabric is a non-woven fabric.

65 8. The abrasion resistant fabric of claim 1 in which the fabric is a knitted fabric.

\* \* \* \* \*